

July 3, 1934.

W. COLVIN, JR

1,965,542

FABRIC

Filed Nov. 24, 1933



FIG. 5

Angle between wrapping strands  
and axis of wire 2

Angle between wrapping  
strands and axis of wire

FIG. 6



-9 INVENTOR  
WILLIAM COLVIN JR.  
By *Auditoria Wood*  
ATTORNEYS

## UNITED STATES PATENT OFFICE

1,965,542

## FABRIC

William Colvin, Jr., Troy, N. Y.

Application November 24, 1933, Serial No. 699,623

12 Claims. (Cl. 117—52)

This application in so far as common subject-matter is concerned, is a continuation in part and in combined form of my application Ser. No. 545,276 filed June 18, 1931, relating to Threads or yarns and fabrics woven therefrom; Ser. No. 563,169 filed September 16, 1931, relating to Threads or yarns and fabrics knitted therefrom; and my application Ser. No. 615,543 filed June 6, 1932, relating to Threads or sewing.

10 The invention relates to threads or yarns composed partially of wire and partially of textile fibers but which are endowed with characteristics of appearance, softness, flexibility, give and resistance to kinking and snarling, fairly comparable to like threads or yarns composed entirely of textile fibers, and which may be used for hand or machine sewing or for the machine production of fabrics, such as by weaving or knitting. It relates particularly to wire threads 15 or yarns which can be used with or interchangeably with threads or yarns composed entirely of textile fibers in any ordinary textile loom, knitting machine or sewing machine, and this without any change or adjustment of the machine. 20 It also relates to fabrics composed entirely of such wire threads or yarns, or partially of such wire threads or yarns and partially of other threads or yarns such as silk, cotton, wool, rayon or the like. My fabrics have the appearance, 25 and to such a substantial degree the characteristics of softness and flexibility, of a fabric of similar weave composed entirely of textile fibers that, generally speaking, it is quite impossible to detect the presence of the wire by a casual examination of the fabric.

Machines can be and have been designed which will weave practically any kind of wire into a fabric. For example, screening, netting, fencing, wire gauze, stiffening fabrics, wire reinforcing, etc., are produced by specially designed machines which weave the wires together. So far as I am aware, however, no one has heretofore been able successfully to produce a wire reinforced thread or yarn of such characteristics that 40 the ordinary mill equipment now used in the textile industries can manipulate the same into cloth and knit goods with the same facility and degree of perfection as pure textile threads or yarns, or which can be used for sewing on an 45 ordinary thread sewing machine.

Wire fabrics made in accordance with my invention have many applications such, for example, as in aircraft, sails, tents, awnings, millinery, upholstering, carpets, rugs, tapes braids curtains, 50 roof and wall coverings, wearing apparel, etc.,

and for general use where extraordinary strength, resistance to stretching and shrinking or electrification of the fabric for heating or other purposes is desirable. They lend themselves particularly to uses where it is desired to simulate 60 in all its characteristics a textile fabric of any well known standard knit or weave and yet have great strength, resistance to stretching or shrinking in one or both directions, electrical heating or a substantially fire proof fabric. Some of my 65 fabrics, for example, can be used for covering the wings of aeroplanes not only because of their extremely high strength but because they may be made substantially fire proof and may be heated by passing a current of electricity through 70 the wires to prevent the formation of ice on the wing surfaces. Similarly, electrically heated garments having all of the softness and flexibility of ordinary cloth fabrics may be made for aviators. As distinguished from the closely woven fabrics, 75 my knitted fabrics may be designed to provide a considerable amount of "give" which particularly adapts them for wearing apparel.

In view of the vast amount of money now invested in weaving, knitting and sewing machinery designed to handle only ordinary textile threads or yarns, and which my invention makes available for the production of wire fabrics, the primary object of my invention may be said to be in providing a thread or yarn having a wire 80 core and which can be used in these already built textile machines for the production of wire fabrics of the same character, with the same facility, and with the same high degree of perfection as the purely textile fabrics which are 85 now produced on these machines.

A further object is to produce fabrics substantially identical with, or very closely approximating in appearance and characteristics, fabrics composed entirely of textile yarns or threads, 90 but in which all or a substantial portion of the structure is composed of threads or yarns having a wire core.

With these and other objects in view, my invention includes the novel thread or yarn and the fabrics made therefrom which are described below and illustrated in the accompanying drawing in which—

Fig. 1 is a highly magnified but not substantially distorted drawing of my thread or yarn 105 in which the core is a #36 wire (B & S gauge) having an actual diameter of 0.005 inches;

Fig. 2 is a view showing how my wire falls 110 limply into a loop without kinking or snarling after it has been subjected to tensile stress;

Fig. 3 is a view similar to Fig. 2 of ordinary magnet wire showing how it kinks and snarls when permitted to become slack after being subjected to tensile stress;

5 Fig. 4 is a magnified and distorted view of a woven fabric in which the entire warp is composed of my wire reinforced threads and the weft of threads composed entirely of textile fibers;

10 Fig. 5 is a fabric similar to that shown in Fig. 4 in which the entire weft is composed of my threads and the entire warp of textile threads;

15 Fig. 6 is a fabric similar to that shown in Fig. 4 in which the warp is composed partially of my threads and partially of textile threads and in which the weft is composed entirely of textile threads;

20 Fig. 7 is a fabric similar to that shown in Fig. 4 in which the warp is composed entirely of textile threads and the weft partially of my threads and partially of textile threads;

25 Fig. 8 is a fabric similar to that shown in Fig. 4 in which the warp and weft is each composed partially of my threads and partially of ordinary textile threads;

30 Fig. 9 is a highly magnified and distorted view of a knitted fabric composed partially of textile threads and partially of my threads; and

35 Fig. 10 is a fabric similar to that shown in Fig. 9 but which is composed entirely of my threads.

Obviously any wire reinforced thread or yarn which can be successfully used in weaving, knitting or sewing machines designed to manipulate only threads and yarns composed entirely of textile fibers must very closely approximate in many of its characteristics a purely textile thread or yarn, otherwise special machines must be designed to manipulate it successfully. In weaving, knitting and sewing, any thread or yarn is subjected to tensile stress at repeated intervals between which it is more or less slack. Ordinary textile thread or yarn does not kink or snarl when so manipulated and any wire thread or yarn which can be successfully used must be comparable with a textile thread or yarn in this respect. Furthermore, a wire thread or yarn must be identical or substantially identical in appearance with the other yarns with which it is knitted or interwoven.

40 For purposes of electrical insulation, it is common practice to cover fine wire with a layer of textile material in the form of threads wound about the wire. Inasmuch as the primary purpose is to cover the wire as efficiently and cheaply as possible, a thread having practically any number of ends can be employed, the greater the number of ends, the quicker the wire can be covered. In order further to insulate the ordinary so-called magnet wire, the surface of the metal is some times coated with lacquer. Very frequently the lacquer is the only insulation used on the wire, but occasionally a lacquer covered wire is also covered with a single layer of cotton or silk thread. The dielectric properties of a coating of lacquer about the wire combined with a single covering of cotton and silk are fully as good if not superior to the dielectric properties of two layers of cotton or silk about the wire and since the power of a magnet depends upon the number of ampere turns the space required for the windings is a very important factor. A thread winding about a wire of the order of #36 or finer practically doubles its diameter. 45 Hence, most magnets are wound from wire hav-

ing only a coating of lacquer thereon because twice as many turns can be made in a given space as with a thread insulated wire. Some are wound with wire having a coating of lacquer and a single layer of cotton or silk thread over the lacquer. So far as I am aware, there was no wire manufactured, prior to my wire, which could be successfully used for knitting, weaving or sewing in an ordinary textile machine. Neither is there any wire manufactured and commercially available which is both coated with lacquer and covered with two layers of textile material in the manner required by my invention in its preferred form. Furthermore, there is no wire commercially available which is inherently corrosion resistant or which has a corrosion resistant surface, other than lacquer, and which is thread insulated. Of course, any wire manufacturer will make wire to any specification, but so-called "double insulated lacquered wire" is not carried in stock and, if obtainable at all, can be had only on special order.

50 Fine, so-called magnet wire wrapped with a single layer of thread cannot be successfully used in textile weaving, knitting and sewing machines. When such a wire is even slightly stressed in tension, the textile covering thereon tends to twist and straighten out. This will be apparent if a piece of such kind of wire, say three feet long, is grasped in the manner shown in Figs. 2 and 3 and pulled taut. As the stress is placed upon the wire, it will be noted that the fibers of the covering which outstand along the wire tend to turn. When the stress is relieved, as shown in Fig. 3, the wire immediately flies into loops, kinks and twists, such as there shown. Such action clogs a textile machine and makes either hand or machine sewing impossible not only because of the kinks but because, once kinked, the wire ruptures under comparatively low tension when again pulled taut.

55 Fine magnet wire wrapped with a double layer of thread is not ordinarily manufactured because of the small demand therefor. Such wire, while not subject to kinking and snarling to the same degree as a single wrapped wire when stressed in tension and relieved, nevertheless does twist, kink and break to such an extent as to render it wholly impracticable for use in a machine designed to manipulate only textile threads or yarns. In these respects it is not substantially better than a wire wrapped with a single layer of thread.

60 I find that this tendency to kink and snarl when relieved of tension, can be overcome by covering the wire with two layers of thread wound in opposite directions about the wire core in such a way that twisting stresses developed when the wire is stressed in tension and relieved, are substantially balanced. When such a double wound wire is stressed in tension, one layer of the covering tends to twist the thread structure in one direction while the other layer tends to twist it in the opposite direction, thus the tendency of the composite structure to twist in either direction is neutralized. In other words the coverings may be said to offer substantially balanced resistances to torsional stresses tending to twist the thread, or to develop torsional strains which are substantially balanced, and the wire or thread, when subjected to tension of the order encountered in manipulating the thread in weaving, knitting and sewing, and relieved, falls limply into a fairly smooth loop as shown in Fig. 2. If very strongly stressed, the loop may merely twist a turn or two but there will be no kinking or snarling.

80

85

90

95

100

105

110

115

120

125

130

135

140

145

150

A wire thread or yarn, according to my invention, must be flexible where it is to be used for sewing, knitting, or in the weft of a woven fabric. In other words the thread or yarn can not be stiff and wiry but must, in its characteristics of softness and flexibility, approximate as closely as possible a pure textile strand of like size. Where it is to be used in the warp of a woven fabric, it may be appreciably less flexible and yet be manipulated by the machine.

In fabricating wire threads or yarns which will not kink and snarl when subjected to tension of the order encountered in weaving, knitting and sewing, and then relieved, so many variable and uncertain factors must be taken into consideration that it seems quite impossible to deduce mathematical formulae which will lead to certain results in all cases.

For example if 120/6 thread (which means a thread of No. 120 size having six parallel ends or strands) is examined under a powerful magnifying glass, it will be found that the separate strands vary considerably in size. Five of the strands may be fairly identical in size while the sixth strand may be very much larger or very much smaller than the others. Again, only four strands may be comparable in size while the fifth is relatively very small and the sixth relatively very large.

While the wrapping threads are generally made with a left twist, they are sometimes made with a right twist, and this is a factor which must be considered because the manner in which the threads lie on the wire depends both upon the twist and upon the direction in which the thread is laid about the wire. For example, a left twisted thread will cling tightly to the wire when wound about it with a left lay but will tend to unwind if wound with a right lay. Likewise a right twisted thread clings tightly when laid to the right about the wire, but with a left lay it is comparatively loose and tends to unwind.

The humidity or moisture in the atmosphere will affect the balance of the wire particularly in the finer sizes to the extent that a wire in substantially neutral balance on an average day may show some degree of unbalance in one direction or the other on a rainy day or on an extremely hot day with low humidity.

Again, the wrapping thread is compressible to a considerable degree and to the extent that a wire of given size may be covered with thread of a given size wound at measurably different pitches.

Depending upon the size of the wire, the tension under which the windings are applied may substantially affect the balance.

Again, the commercial threads which are obtainable are sizes 120, 100, 80, 60 etc. These are obtainable with substantially any number of ends or strands but obviously not in fractions of strands. Hence, if mathematical calculations indicated that to obtain a theoretically desirable pitch ratio in the upper and lower windings a No. 120 thread having 5.5 ends should be used in the first wrapping, with a No. 100 thread having 6.5 ends in the top, it would be necessary to compromise on a 5 or 6 end bottom with a 6 or 7 end top depending on which gives or should give the best balance.

It must be borne in mind that except in the finer sizes, say #30 gauge and finer, accurate theoretical balance is not so essential. Perhaps it would be more accurate to say that where the thread is not slightly stretched or elongated in

manipulating it into a fabric, or in sewing, balance is not so necessary, because without stretching there is no tendency of the windings to twist and kink the wire. The wire thread need be balanced only to the extent that it will not kink or snarl when subjected to tension of the order encountered in the weaving, knitting or sewing operations in which it is to be used, and then relieved. Obviously, the finer the wire core the more the thread or yarn will elongate during the manipulation thereof, and hence, as a general rule, it may be said that the finer the thread the finer the balance required. Moreover, the coarser the wire the more inherent resistance it has to twisting, kinking and snarling.

As a specific example of my thread or yarn I will show below the effect of winding a #36 wire in various ways. The thread employed was a left twist cotton both in the bottom and top layers, and the bottom winding was a right lay and the top winding a left lay in all cases.

It should be noted that in the case of a wire wound with a single right-lay wrapping when slightly stressed in tension and permitted to fall into a loop as shown in Fig. 2, the loop, when observed from above the hands, will turn or twist in a clockwise direction, whereas a single left-lay wrapping will cause the loop to twist counter-clockwise. Hence, if a loop of wire wound with a right-lay bottom and left-lay top twists clockwise it is due to what may conveniently be termed an over balance in the lower winding, and if it twists counter-clockwise, it is due to an over balance in the upper winding.

In the following table  $a_1$  is the pitch angle of the helix of the inner winding, and  $a_2$  is the pitch angle of the helix of the outer winding. These were determined quite accurately by cutting a six inch length of thread and unwinding and measuring the length of the inner and outer thread layers thereon. From these measurements the pitch angles  $a_1$  and  $a_2$  were calculated.

| Specimen | $a_1$   | $a_2$   | Ratio<br>$\tan a_2$<br>$\tan a_1$ | Thread |       | 120   |
|----------|---------|---------|-----------------------------------|--------|-------|-------|
|          |         |         |                                   | Bottom | Top   |       |
| A        | 63°-14' | 47°-20' | 0.5473                            | 120/6  | 120/6 | 120/6 |
| B        | 61°-09' | 43°-17' | 0.5188                            | 120/6  | 120/6 | 120/6 |
| C        | 59°-41' | 47°-48' | 0.6448                            | 120/6  | 120/6 | 120/6 |
| D        | 60°-7'  | 47°-2'  | 0.6238                            | 120/6  | 120/6 | 120/6 |
| E        | 57°-37' | 43°-14' | 0.5962                            | 120/6  | 120/6 | 120/6 |
| F        | 59°-41' | 43°-55' | 0.5630                            | 120/6  | 120/6 | 120/6 |
|          |         |         |                                   |        |       | 125   |

Of the above specimens, A is nearly perfectly balanced. On slight tension it showed a very slight bottom overbalance, while as the tension was increased the overbalance changed to a slight top overbalance to the extent that the loop made one turn counter-clockwise.

Specimen B indicated a very bad bottom overbalance to the extent that the loop flew into kinks and snarls. It is entirely unsuitable for sewing, weaving or knitting.

Specimens C and D both indicated a very bad overbalance in the top. These threads were practically as much out of balance as specimen B and are entirely unsuited for weaving, knitting or sewing.

Specimen E, when examined under a magnifying glass, indicated comparatively wide gaps in the outer winding, estimated as having a width of from one to two threads, so that its general appearance was much like a barber pole. However, this thread showed only a moderate top overbalance and, in this respect, is quite well balanced.

suited for weaving, sewing and knitting. Although not as good as specimen A, it did not kink or snarl.

Specimen F showed a slight overbalance in the top but is practically as well if not better balanced than specimen A and is well suited for weaving, sewing and knitting.

From the foregoing it will be apparent that for a No. 36 wire core very slight changes in the relative pitches of the inner and outer windings substantially affect the balance of the composite thread. The difference between specimen A and specimen B is only about  $4^{\circ}$  in the top and  $2^{\circ}$  in the bottom, yet A is good, whereas B is hopelessly bad. Likewise specimen B does not differ substantially from specimen F in the top wrappings and there is something less than  $2^{\circ}$  difference in the bottom wrappings yet F is a very well balanced thread.

20 In practice, the following procedure is recommended to produce a balanced thread.

The lacquered or enameled wire is drawn upwardly through an insulation winding machine adapted to apply simultaneously the inner and outer thread wrappings in opposite directions about the wire. If a No. 36 wire is being covered with a No. 120/6 thread in the lower layer and a No. 120/6 thread in the upper layer, the pitch angle at which the first wrapping is applied should be adjusted so that the wire is well covered as it advances, and the pitch angle at which the second wrapping is applied should be adjusted so that the inner wrapping is smoothly covered by the outer wrapping. These angles will probably automatically work out to be between  $55^{\circ}$  and  $65^{\circ}$  for the inner winding and between  $40^{\circ}$  and  $50^{\circ}$  for the outer. It is not necessary to know their precise values and it is only required that both wrappings effect a good coverage.

40 As the wrapped wire passes from the machine, break off a three foot length and subject to fairly good tension by pulling with the hands and then permit it to fall into a loop as shown in Figs. 2 and 3. If the wire is very much out of balance, it may be necessary to try a very light tension on the first tests otherwise, when relieved, it will fly so quickly into kinks and snarls that it will be quite impossible readily to determine which way the loop twisted.

50 As the wire falls into the loop, note which way the loop twists. If clockwise, it indicates an overbalance in the bottom winding, and if counter-clockwise, an overbalance in the upper winding. The pitch at which one or both of the windings is being applied should then be changed very slightly to correct for this unbalance. Generally, decreasing the pitch angle of the inner helix or increasing the pitch angle of the outer helix will correct an overbalance in the lower winding. Likewise, generally, increasing the pitch angle of the inner helix or decreasing the pitch angle of the outer helix will correct an overbalance in the outer winding.

60 After changing the pitch angle of one or both of the windings repeat the loop test and again adjust the pitch angle or angles to correct any overbalance which is sufficient to cause pronounced snarling or kinking when the thread is subjected to tension of the order encountered in the use—sewing, weaving or knitting—to which it is to be put, and then relieved. Repeat the test and adjust if necessary.

70 In applying the thread wrapping it is extremely desirable that the tension on the thread be so regulated that the wire itself is not distorted

to the extent that the wire and thread are twisted together instead of the thread being wrapped smoothly about the wire. This frequently occurs in ordinary magnet wire and, as a result thereof, the finished wire is very stiff and springy and in no way resembles a textile thread. I prefer that no more tension be employed on the thread wrappings than is necessary to obtain a good even coverage.

80 Where my wire thread or yarn is being supplied to a textile mill in which the weaving or knitting operations are conducted in an atmosphere of constant humidity, the thread may be manufactured and balanced in an atmosphere of the same humidity so that an ideal thread is thus obtained.

85 The pitch at which the windings are laid affects the flexibility of the wire as will be apparent from a consideration of what occurs when the thread is flexed as a beam, bearing in mind that while a fine thread offers slight resistance to bending it does, nevertheless, offer appreciable resistance to tensile stress. Where the wrappings are laid at a comparatively flat pitch or at a large angle to the axis of the wire the convolutions of the wrappings on the side of the wire which is subjected to tension tend merely to separate. In other words, the strands of the covering are not subjected to tensile stress and therefore do not appreciably resist the bending. On the other hand, where the wrappings are laid at a comparatively steep pitch or small angle with the wire axis, the strands of the wrapping, instead of separating on the side of the wire which is subjected to tensile stress to the same degree as flat pitch windings, are themselves stressed in tension and thus tend to increase the resistance of the wire to bending. For this reason, it is desirable to attain a balanced thread by selecting as flat pitch angles for the inner and outer helices as is consistent with economical production. These angles, of course, may be varied considerably by varying the number of ends in the wrappings. Generally, it is not necessary to use less than five ends in the first wrapping to attain the desired result, and once the pitch angle of the first wrapping is fixed, the number of ends and the size of thread used in the outer wrapping is more or less fixed by the necessity of covering the inner wrapping and at the same time balancing the thread.

100 While I prefer to attain the desirable kink and snarl resisting characteristics of my thread by adjusting, as pointed out above, the pitches, or either of them, at which the windings are applied it is to be understood that my invention is not limited to this method of procedure. Any thread having two wrappings wound in opposite directions about the wire core and which indicates, when subjected to the "tension and loop" 110 test above described, that it is decidedly unbalanced, may be made resistant to kinking and snarling by first subjecting it to sufficient tension to effect a slight permanent elongation or stretching, and then permitting the torsional 120 strains thus developed in the thread to relieve themselves by twisting the thread axially in the proper direction while it is maintained under sufficient tensile stress to prevent looping. A thread so treated will not kink or snarl when 130 again subjected to tensile stress of the order required to effect the elongation and then subjected to the loop test. However, thread which has thus been stretched beyond the elastic limit of the wire core lacks, to a considerable degree, 140

145

150

155

160

165

170

175

180

185

190

195

200

205

210

215

220

the soft, yielding, elastic characteristics of 46% solvent, and having a specific gravity of about 0.90.

Inasmuch as my thread or yarn for universal use is subjected to severe bending, it is quite essential that the varnish coating employed be extremely flexible so that it does not appreciably effect the flexibility of the wire. Moreover the varnish should be of such character that it will not crack or flake when the finished thread or yarn is bent about a mandrel of its own diameter.

80

85

90

95

100

105

110

115

120

125

130

135

140

145

150

While my invention is not limited to the copper wire alone, I find that this metal can be readily processed to adapt it for weaving, knitting and sewing, and that excellent fabrics can be made therefrom on ordinary machinery designed to handle only pure textile material. Where the thread is to be used for knitting, sewing and in the weft of the fabric, the metal in the core should have characteristics of strength, 10 flexibility and ductility reasonably comparable with commercially pure annealed copper. Irons and low carbon steels, for example, can be soft annealed to have these desirable characteristics, and these and any other metals or alloys in which 15 these physical properties are inherent, or which can be processed to endow the wire drawn therefrom with these characteristics, can be used. Where the wire is to be used in the warp, flexibility is not such an important factor, except 20 insofar as it affects the character of the finished goods, and for this reason wire which is very much less flexible than copper can be employed.

In the finer sizes great care should be exercised in the wire drawing process to insure that 30 the metal core is absolutely uniform in cross section throughout. Uniformly low or moderate drawing speeds with a gradual reduction to the desired size, are recommended, as distinguished from the relatively high, non-uniform speeds 35 and quick reduction to size which characterizes the production of ordinary magnet or other wire not intended to be subjected to substantial tensile stress. Weak spots in the core itself, if they do not cause rupture, permit the thread to stretch 40 or elongate to a greater degree in the zones thereof than elsewhere, thus unduly stressing the windings about these spots and cause kinking.

For universal use, however, the wire is preferably made of commercially pure copper or a metal which has or can be processed to have the 45 desirable characteristics of copper. For sizes 32 (B. & S gauge) and finer, the copper wire is drawn down very carefully from size 22 to insure absolute uniformity in size and is thereafter 50 pot annealed at a temperature from 600° F. to 750° F., according to size, for a period of from 1½ to 2 hours. After the heating treatment, the pots are sealed and the wire is allowed to "soak" until the temperature reaches 90° F. to 55 100° F., which ordinarily will require from 15 to 18 hours. This treatment should produce a wire having a minimum elongation of about 25%.

Inasmuch as copper is not highly resistant to 60 corrosion and many fabrics in the course of normal use will be washed or otherwise subjected or exposed to corrosive agents, I next give the wire a protective film or thin coating of varnish or enamel which must be of such character that it 65 will provide a hard, tough, elastic covering for the wire. Where the fabric is to be "electrified" the enamel should also possess high dielectric properties.

A very excellent varnish or lacquer may be made 70 by combining China wood oil, rosin ester, lead dryer and kerosene, but other materials which will produce a varnish having the physical characteristics above mentioned may be used. The above ingredients are mixed to produce a varnish 75 containing about 54% solids and approximately

the soft, yielding, elastic characteristics of 46% solvent, and having a specific gravity of about 0.90.

Inasmuch as my thread or yarn for universal use is subjected to severe bending, it is quite essential that the varnish coating employed be extremely flexible so that it does not appreciably effect the flexibility of the wire. Moreover the varnish should be of such character that it will not crack or flake when the finished thread or yarn is bent about a mandrel of its own diameter.

To produce the specially flexible coating required for my thread, the varnish should be applied by successive passes through a bath and baking oven. For example, the wire may be given four separate coats of varnish and, after each coat, run through a six foot oven at a temperature of from 750° F. to 800° F., and at a speed of 60 to 80 feet per minute depending somewhat on the size of the wire being coated. The thickness of the coating may vary from say 0.00015 to 0.0005 inches depending upon the size of the wire.

Referring to Fig. 1, 7 is the wire core coated with the enamel 8. After coating with enamel the wire is covered, in the manner described above, with two layers or wrappings of fibrous material such as thread of silk, cotton, rayon, wool or the like depending upon the character of the fabric desired and, where the fabric is to be electrified, upon the insulation required. The outer layer is always laid in a reverse direction to that of the inner layer and is preferably always a left hand lay so that it will cling tightly to the wire when ordinary left twisted thread is used for the winding. In Fig. 1, 9 represents generally the inner layer of wrapping which, in the case of the 110 finer sizes of wire such as the No. 36 here shown, may comprise five or six ends 9'.

Bearing in mind that in wire of the finer sizes the first wrapping of thread approximately doubles or more than doubles the diameter of the 115 wire and that it is quite essential, in order to prevent kinking and snarling, that the inner and outer layers of wrapping offer substantially balanced resistances to torsional stresses developed by tension on the thread, it may be necessary or desirable to use more or less ends in the outer wrapping than in the inner wrapping in order to attain this result and completely cover the inner wrapping.

Where necessary or desirable, the fibrous covering may be impregnated with suitable compounds, but the finished wire should have a smooth polished surface. As a matter of fact it is recommended in any case, after the coverings have been wrapped about the wire, that the wire 125 be run through dry cloth wipers to bring about flattening and smoothing of the outer covering.

In many instances, especially in the weaving of heavy-bodied, ribbed fabrics, such as corduroys, velvets, pluses etc., a wax-impregnated wire 135 thread while not absolutely essential is extremely desirable from a practical standpoint because the weaving process is greatly facilitated thereby. If desired, after the fabric is woven, the wax may be removed by ordinary washing or, depending 140 upon the character of the wax, by the use of appropriate solvents.

For example, to provide a very smooth, slick surface, or, for insulating purposes, the wire may be run through a bath comprising about 35% of 145 light carnauba wax, 15% of white finishing wax with a paraffine base, and 50% of regular paraffine wax with a melting point of around 130° F. The bath mixture should be heated to around 220° F. and the wire speed may be about 70 feet per 150

minute. As the wire emerges from the bath, it should be carefully wiped and polished to provide a uniformly smooth surface finish. Three felt wipers advantageously placed may be employed, the first to remove the surplus compound, the second to remove the roughness, and the third to smooth and polish the coating.

Where flame resisting characteristics are desired, the fibrous material may be impregnated with "Halowax", which consists of chlorinated naphthalene, or with a compound made up of oxidized stearine pitch.

In preparing my wire for use in the loom it is first spooled in continuous lengths. The required number of spools corresponding to the number of individual strands or wire in the fabric are then placed on racks, each spool having its own spindle upon which it may turn freely. The ends of the wire are taken from the spools and around two cylindrical tension bars, each successive end being taken around the bars in the opposite direction to the next end. From the tension bars the wires are led to and wound on the beam by power, the previously mentioned tension devices providing a smooth uniform wind on the beam. The wires are uniformly spaced on the beam by means of reeds and the ends of the wires are tied to a reed secured to the beam so that threading into the loom is facilitated.

Where the metal or alloy of which the wire is made is resistant to corrosion and the enamel coating is not needed for electrical insulation, it may be omitted. Likewise, where staining of the fabric due to corrosion of the copper is immaterial, the enamel coating may also be omitted.

For purposes of illustration only, I have shown in Figs. 4, 5, 6 and 7 a typical duck or twill weave and although these drawings indicate that the fabric is of open texture it is to be understood that this is merely for purposes of clearness and that in the fabrics as actually woven the strands are very close together and the fabric is in all respects identical in appearance with ordinary duck or twill composed entirely of textile threads. In Figs. 4, 5, 6, 7 and 8 the vertical strands indicate the warp in each case and the horizontal strands the weft.

In Fig. 4 the warp strands 11 are made of my thread while the weft strands 12 are of textile thread.

In Fig. 5 the warp strands 13 are of textile threads and the weft strands 14 are of my wire threads.

In Fig. 6 the alternate warp strands 15 are wire threads and the other warp strands 16 are of textile threads while the weft threads 17 are of textile threads.

In Fig. 7 all of the warp strands 18 are of textile threads while wire threads 19 and textile threads 20 alternate in the weft. In Fig. 8 wire strands 21 alternate with textile strands 22 in the warp and wire strands 23 alternate with textile strands 24 in the weft.

Although I have not shown any fabric in which the entire warp and weft is composed of wire, it is to be understood that it is perfectly possible to weave such a fabric. Furthermore, it is to be understood that my wire threads are adapted for making any kind of woven cloth.

In Figs. 9 and 10 I have shown knitted fabrics which for the purposes of clearness are shown as greatly enlarged and distorted to the extent that the fabrics appear to be open. Actually these fabrics may be as closely knitted as any knitted fabric composed entirely of textile yarn.

In Fig. 9 I have shown one of my threads 25 interknitted with textile yarns 26 and 27 while in Fig. 10 I have shown a knitted fabric composed entirely of wire reinforced yarns 28.

It is to be understood that my covered wire is intended primarily for use in instances where it is subjected to tension of the order encountered in hand and machine-sewing and in textile machinery, and where, in the use of wrapped wire there would be a substantial tendency for it to kink or snarl. Hence, to avoid excessive verbiage, the term "textiles", as used in the claims, is to be understood as including textile fabrics and structures of the character ordinarily composed only of pure textile fibers and made or stitched, or which can be made or stitched, on or by ordinary looms, knitting machines, or sewing machines designed to manipulate only threads or yarns composed entirely of textile fibers, as distinguished from fabrics and structures which can not be so made, although it is to be understood that the claims are to be interpreted as including thread for hand stitching. The terms "textile machine" and "textile machinery" are to be deemed as including sewing, knitting and weaving machines of the type ordinarily employed in the manipulation of pure textile threads or yarns, as distinguished from such machines especially designed to manipulate wire. Likewise the term "thread" is to be understood as including "yarn".

What I claim is:

1. As a new article of manufacture, thread for use in sewing and fabricating textiles, and which can be used in textile machinery with substantially the same facility as thread composed entirely of textile fibers, comprising a ductile, easily flexible metal wire core enclosed in wrappings of textile thread including two layers laid in opposite directions on the said core, said wrappings being so laid and correlated as to develop substantially balanced torsional strains when subjected to tension effecting a permanent elongation of the core; whereby correlative action of the wrappings substantially overcomes the tendency of any portion of the composite thread to kink or snarl after the release of tension thereon.

2. As a new article of manufacture, a thread for use in sewing and fabricating textiles, comprising a ductile, easily flexible, substantially inelastic core of a character to become permanently elongated when subjected to tension, said core being enclosed in two layers of wrappings of flexible character laid in relatively opposed directions on the same, said wrappings being so laid and correlated as to develop substantially balanced torsional strains when subjected to tension effecting a permanent elongation of the core; whereby correlative action of the wrappings substantially overcomes the tendency of any portion of the composite thread to kink or snarl after release of tension thereon.

3. As a new article of manufacture, a thread for use in sewing and fabricating textiles and which can be used in textile machinery with substantially the same facility as thread composed entirely of textile fibers, the same including a ductile, easily flexible metal wire core enclosed in layers of wrappings of flexible character laid on the said core in relatively opposed directions, said wrappings being so laid and correlated as to develop substantially balanced torsional strains when subjected to tension effecting a permanent elongation of the core; whereby correlative action of the wrappings substantially overcomes the tendency

- of any portion of the composite thread to kink or snarl after release of tension thereon.
4. The structure set forth in claim 3 in which the surface of the wire is resistant to corrosion.
5. A fabric comprising as an essential portion thereof thread in accordance with claim 3.
6. A fabric comprising as an essential portion thereof thread in accordance with claim 3, in which the surface of the core of said thread is resistant to corrosion.
7. A woven fabric comprising as an essential portion thereof thread in accordance with claim 3.
8. A knitted fabric comprising as an essential portion thereof thread in accordance with claim 3.
9. A fabric composed substantially entirely of thread in accordance with claim 3.
10. A woven fabric characterized by a substantial portion of the warp being composed of thread in accordance with claim 3.
11. A woven fabric characterized by a substantial portion of the weft or filler being composed of thread in accordance with claim 3.
12. As a new article of manufacture, a fabric having the appearance and, to a substantial degree, the characteristics of softness and flexibility of a fabric of similar structure composed entirely of textile threads and made by textile machinery, characterized by being formed in substantial part of thread having a fine, substantially inelastic, easily flexible, ductile metal wire core enclosed in a plurality of layers of wrappings of textile thread wound on the core in relatively opposed directions, said wrappings being so laid and correlated as to develop substantially balanced torsional strains when subjected to tension effecting a permanent elongation of the core; whereby correlative action of the wrappings substantially overcomes the tendency of any portion of the composite thread to kink or snarl after release of tension thereon.

WILLIAM COLVIN, JR.

25

100

30

105

35

110

40

115

45

120

50

125

55

130

60

135

65

140

70

145

75

150

80

85

90

95